

G. A. HENDERSON

PLASTIC COMPOSITION AND PROCESS OF MAKING SAME.  
APPLICATION FILED NOV. 30, 1914.

1,187,314.

Patented June 13, 1916.

2 SHEETS—SHEET 1.



G. A. HENDERSON.

PLASTIC COMPOSITION AND PROCESS OF MAKING SAME.

APPLICATION FILED NOV. 30, 1914.

1,187,314.

Patented June 13, 1916.

2 SHEETS—SHEET 2.

Fig. 2.



Fig. 6.



Fig. 5.



Fig. 4.



Fig. 3.



Witnesses:

John A. Henderson  
M.C. Jenkins

Inventor:

George A. Henderson

# UNITED STATES PATENT OFFICE.

GEORGE ASA HENDERSON, OF ST. ALBANS, WEST VIRGINIA.

## PLASTIC COMPOSITION AND PROCESS OF MAKING SAME.

1,187,314.

Specification of Letters Patent. Patented June 13, 1916.

Application filed November 30, 1914. Serial No. 874,934.

*To all whom it may concern:*

Be it known that I, GEORGE A. HENDERSON, a citizen of the United States, residing at St. Albans, in the county of Kanawha 5 and State of West Virginia, have invented certain new and useful Improvements in Plastic Composition and Processes of Making Same, of which the following is a full, clear, and exact description, reference being 10 had to the accompanying drawings, forming a part of this specification.

The invention relates to a plastic composition and process for making the same, with especial reference to the treatment of 15 woody particles and the manner of their incorporation with a preservative binder in the production of improved paving material to constitute the upper or wearing surface of paving structures and my object is 20 to provide permanent density and resiliency in such structures.

In carrying out the invention, woody fiber, preferably that of hard wood, is prepared by shredding billets of wood into particles of 25 various sizes and shapes, and the removal from the particles of all sap, pulp and all other matter than a plurality of woody fibers forming each particle by first boiling, retting, steaming, or other method known to the 30 trade, simultaneously abnormally enlarging the pores of the particles, followed by the discharge of the major portion of the moisture therefrom, then grading the particles as to sizes to substantially reduce the voids 35 between them, then mixing the particles in a vat with a preservative-binder to preserve the particles and to bind them to each other, simultaneously applying to the mass, when mixing in the vat, severe and continuous 40 heat to exhaust, or to completely develop, the absorbing efficiency of the particles, simultaneously partially filling the pores therewith, when abnormally enlarged and then completely filling them by entrapping, 45 when cooling, and contracting the binder of a preservative nature, which is applied in quantity predetermined in exact relation to the known extent of the pores within, and voids between, the particles, which are pre- 50 measured by determining the degree of their expansion from normal and contraction to normal size, and on this basis fixing the quantity of such preservative-binder to be mixed with the particles in one operation as 55 exactly sufficient to completely fill said

pores, when contracted, to coat the particles, to fill the voids between them when compressed, and to bind them to each other, all in the manner hereinafter described, for the purpose of rendering the completed product 60 of permanent, fixed size, density and resiliency, and, therefore, less susceptible to subsequent expansion and contraction by the action of the elements than are such compositions containing vegetable fiber not so 65 treated.

The nature of my invention will be best understood by reference to the accompanying drawings which will now be described, it being premised, however, that various 70 changes may be made in the apparatus by which the process is carried out, without departing from the spirit and scope of the invention as defined in the appended claims.

In the accompanying drawings, Figure 1 75 is a view partly in side elevation and partly in vertical section of an apparatus adapted for carrying out the invention. Figs. 2, 3, 4, 5 and 6 are cross sections through pavements embodying the product of the invention 80 and having been made by the process.

Referring to the drawings by numerals, 2 indicates a chipping, grinding or shredding mill for wood billets, the mill being driven by shaft 4 actuated by pulley 3. A spout 5 delivers the particles of wood of various sizes and shapes to the vat 6 in which the particles are placed. Vat 6 is provided with steam pipe 7 through which steam is admitted for heating the material within 90 the vat and to extract the juices, and pulp from the particles and to abnormally enlarge the particles. The matter thus loosened from the wood fibers and extracted therefrom is drawn off from time to time 95 through outlet cock 8 and may be used in any preferred way as a by-product.

A drying oven 9 is suitably located relative to vat 6 and is provided with a plurality of endless conveyers 10, 11 and 12, which 100 pass about drums 13, conveyer 10 being extended past the lower or discharge end of a supply duct 19 in which the particles are placed when taken from vat 6, whereby the particles may be readily deposited from 105 vat 6 through valve 20 onto the conveyer 10. In the lower portion of the drying oven is arranged the gas supply pipe 15 having a burner 16 adapted to supply the heat for the oven. The products of com- 110

bustion starting from this heater pass upward through flues 17 and thence out to the stack 18. The flues 17 extend between the endless conveyers and are connected at their ends by cross flues so that the products of combustion have a back and forth passage from the heater to the discharge stack whereby the major portion of the moisture is removed from the particles, though in this step in my process the moisture content of the particles may be, when omitted from this drier, as high as from seven to twelve per cent. Conveyer 12 discharges onto a screen 14 arranged within the chamber 19<sup>a</sup> forming part of grading machine which will now be described. Hot air from steam pipes 19<sup>b</sup> is removed from chamber 19<sup>a</sup> by the operation of fan 19<sup>c</sup> for carrying off a portion of the impalpable powder so that the material passing through the screen 14 will thereby be rendered free from an impractical quantity and then contain not more than two or three per cent. of such powder. Those particles of fibrous material which fail to pass through the mesh of screen 14 are delivered from the end of the screen to the mill 14<sup>a</sup> where they are ground and delivered to a conveyer 14<sup>b</sup> which in turn returns them to the screen 14.

Discharging from the chamber 19<sup>a</sup> the particles are delivered to the successive screens 21<sup>a</sup>, 21<sup>b</sup>, and 21<sup>c</sup> of grading machine 21 of different mesh for separating the particles according to size, into four separate predetermined grades thereof descending from those in sizes, when dry  $4x\frac{1}{2}$ " as the largest, to impalpable dust, in the manner, viz.: Screen 14 is provided with mesh which will permit the passage into chamber 19<sup>a</sup> of particles of the size that will pass a square mesh one quarter of one linear inch in diameter, and be retained on a ring one half of one inch in inside diameter, and graduating from that size on down to impalpable dust, all particles to be used passing this mesh. In practice I prefer to use screens of the shaker type to those of the revolving type, known to the trade. The shaking of the screens 14, 21<sup>a</sup> and 21<sup>b</sup> results in the larger particles thereon being worked to the top of the mass of particles in the screens whose mesh will not permit their passage through them. Screens 21<sup>a</sup> and 21<sup>b</sup> contain mesh in a scale descending from that of the mesh in screen 14, and by reason of the inclination of these screens from horizontal the particles which will not pass them are, by the operation of these screens, deposited into the re-grinder, in the first instance and then into the measuring boxes, separate from, and in relatively smaller quantity than the grade that passes screen 21<sup>c</sup>. All of the particles which reach screen 21<sup>c</sup> pass its mesh, and are likewise

conveyed to measuring box 21<sup>b</sup>, as shown in the drawing, in greater quantity than, and separate from the other grades. Accordingly the mesh in screen 21<sup>c</sup> is preferably of a size midway between the size of impalpable dust and the largest particles, above mentioned, or viz.,  $1\frac{1}{2}x\frac{1}{2}$ ", screen 21<sup>c</sup> being midway between the latter size and the largest mesh of screen 14, or of a size  $\frac{3}{16}x\frac{3}{8}$ ", while screen 21<sup>c</sup> is designed to pass all chips which pass screen 21<sup>c</sup>, and is of the size mesh  $\frac{1}{16}x\frac{1}{4}$ ". It will therefore be obvious by reference to the drawing that the particles which pass screen 14 will be in sizes graduating in descending scale from those  $4x\frac{1}{2}$ " to dust; those that pass screen 21<sup>a</sup> being of the sizes  $1\frac{1}{2}x\frac{3}{8}$ " graduating in descending scale to dust, while the particles of the sizes between  $1\frac{1}{2}x\frac{3}{8}$ " and the size  $\frac{1}{16}x\frac{1}{4}$ " are separated from the sizes that pass screen 21<sup>c</sup>, and conducted to measuring box 21<sup>b</sup>. Likewise the particles of the sizes between  $1\frac{1}{2}x\frac{3}{8}$ " and  $\frac{1}{16}x\frac{1}{4}$ " are so separated and conducted to measuring box 21<sup>b</sup>, while the sizes graduating from  $\frac{1}{16}x\frac{1}{4}$  down to dust are passed by screen 21<sup>c</sup> and conveyed to measuring box 21<sup>b</sup>, in which measuring boxes, 21<sup>b</sup>, the three grades, in addition to the relatively small percentage of impalpable dust remaining, are measured in such predetermined quantities of each grade, that when mixed together the resultant volume of their aggregate will be equal to from seventy to ninety per cent. of their aggregate volume before being so graded, depending on the nature of the wood selected for use in the carrying out of the process. In practice I have discovered that to accomplish this degree of reduction in voids between the particles they shall be graded in sizes as follows: The particles in sizes  $4x\frac{1}{2}$ " to  $1\frac{1}{2}x\frac{3}{8}$ ", 15%; those in size  $1\frac{1}{2}x\frac{3}{8}$ " to  $\frac{1}{16}x\frac{1}{4}$ ", 15%; those in size  $4x\frac{1}{2}$ " to impalpable dust, 68%, impalpable dust 2%. The particles are then delivered in the proper practical percentages of each of the particles of various sizes to the common discharge tube 21<sup>c</sup> which discharges into hopper 22<sup>a</sup> communicating with the mixing tank 22.

Simultaneously a preservative of a cementitious nature, hereinafter described, heated in kettle 21<sup>c</sup> to a temperature of from 250 to 300 degrees Fahr., is delivered through measuring box 21<sup>b</sup> into hopper 22<sup>a</sup> in quantity hereinafter prescribed, and the mass is then agitated in the presence of heat within vat 22, which is open at its hopper 22<sup>a</sup> and mouth 22<sup>b</sup>. For the purpose of such agitation of the mass of particles and binder in vat 22, a central shaft 22<sup>c</sup> extending longitudinally through vat 22 is provided with agitating blades 22<sup>d</sup>, 22<sup>e</sup>, anchored thereto, and revolved by the operation of shaft 22<sup>c</sup> and pulley 22<sup>d</sup>, which blades are so shaped

as to agitate and to move the material from the direction of the hopper 22<sup>a</sup> toward, and to be emitted from, the mouth 22<sup>b</sup>. In this mixer 22, which may be of any approved mechanism, in which all of the ingredients forming the composition are placed and mixed simultaneously, the mass is sufficiently heated, to-wit: to 250 degrees Fahr., and agitated a sufficient length of time to exhaust, or to completely develop, the absorbing efficiency of the particles, simultaneously absorbing the molten preservative-binder with which they are mixed, the quantity thereof being predetermined, as herein after described, to only be sufficient to partially impregnate the expanded pores of the particles. When the mass is, in said mixer, at a temperature of approximately 250 degrees Fahr., and after it has been sufficiently agitated and heated a sufficient length of time to accomplish the purpose aforesaid, it is removed from the vat and spread on a previously prepared road base to a thickness of not exceeding four inches. While the particles are then contracting from their hot volume to their cold volume under the influence of atmospheric temperature, thereby entrapping the contained binder, with which they are surrounded, to the extent of completely filling the pores therewith when so contracted, the mass is gradually compressed to the extent of causing some of the hot preservative-binder to be emitted from the particles pores to act as a binder of the particles in the completed product; only sufficient compression being applied to the hot mass to effect the complete filling of the pores and voids, and the practical dissemination of the melted binder throughout the particles and throughout the thickness of the mass, to-wit: approximately one half of its initial thickness, without squeezing to the outer edges, or top of the compressed mixture any more preservative than exists throughout the depth and area of the product, but sufficiently to cause the binder to partially exude from the contracted pores to fill the voids between the compressed particles, and to bind them to each other. The mass may be emitted from the mixer and baled for storage and shipment into bales approximately 3 ft. x 5 ft. in which event it shall be reheated to approximately 250 degrees Fahr., before being spread on the road and compressed.

The preservative-binder to be used in my process consists of a wood-preservative of a binding nature, preferably plastic bitumen known to the trade, consisting of a natural or artificial asphalt, coal-tar or pitch composition, in which the oily constituent is reduced to the minimum, the volume of the composition of bituminous nature, in relation to the weight thereof being predetermined in relation to that of the woody par-

ticles as hereinafter described. A coating of such a binder may be spread over the surface and covered by a thin layer of hot sand sprinkled thereon. This coating, when used, is applied after compression is begun 70 and before completed.

The quantity of binder and filler of the pores and voids is to be determined by first thoroughly drying a quantity of the particles to be used, from which particles have 75 been removed such matter as sap, pulp and moisture, the particles so graded and the pores thereof so abnormally enlarged that the pores within and the voids between them aggregate from 40% to 70% by volume of 80 their mass and, in any well known manner, determining the extent of the voids and pores present within the un-contracted, un-compressed mass of graded, dry wood particles; and then determining, by actual experiment, the degree to which the particles can be contracted and compressed, when mixed with the hot preservative binder, and the mass agitated in the presence of heat, and then noting the extent of reduction by 85 volume from that of the hot, abnormally enlarged woody particles, and of the hot preservative, and of the hot mass of the two mixed together, to that volume of the same mass when cooled, subsequently, under the 90 gradual compression herein described.

The preservative forms the binder for the material. In this connection it must be remembered that a binding agent, or adhesive, has no binding value until the particles 100 sought to be bound thereby have completely used up or expended the whole of their absorbing efficiency.

In practice, after determining the volume of voids and pores to be filled with the preservative-binder, and after determining the quantity necessary to exactly fill them when contracted and compressed, and to fill the voids between the particles when contracted and compressed to the extent herein prescribed, I prefer to add to that quantity, before mixing the ingredients, approximately from seven to ten per cent. of the same preservative-binder, to act as the binding agent in the completed product. In this manner 105 is the product rendered comparatively free from voids, or from an impracticable excess of preservative or binder. In my use of chestnut wood I have found that such voids and pores, when so treated, and when thoroughly dried and graded, but before being mixed with their preservative-binder, and before compressed, approximate sixty-seven 110 per cent. of the aggregate volume thereof, while in my use of quebracho wood and 115 other hardwoods the porosity of the particles, and voids between the aggregate particles, are equivalent to from forty to 120 seventy per cent. of such volume.

In my process, the proportions to be em- 125

ployed, of pitch, of natural or artificial asphalt or other bitumen, depend on the nature of the wood employed as well as the nature of the preservative-binder, when treated according to my process, viz: I prefer the particles of hard wood, and I have obtained excellent results from chestnut wood particles, in which the particles were so treated, their pores so enlarged, and the particles so dried and graded that two hundred cubic feet thereof, when uncompressed, weighed two thousand pounds; the preservative binder employed being of natural asphalt which was so treated, that two thousand pounds of said asphalt unheated, measured thirty-three cubic feet in volume. The basis of sixteen and two-thirds per cent. of one cubic foot of this treated asphalt, measured cold, and mixed hot with one cubic foot 20 of said uncompressed, dried and graded chestnut wood particles, resulted in the aggregate of one-half of one cubic foot of mixed material, contracted and compressed in the completed product, in which were present thirty-three per cent. by volume and fifty per cent. by weight of asphalt, with sixty-seven per cent. by volume and fifty per cent. by weight of comparatively uncontractile, uncompressible solid wood matter, the remaining voids in this completed pavement being less by volume than in any other pavement of which I have knowledge.

In practice I have discovered that the proportions to be practically mixed vary according to the nature of the wood and the degree of its susceptibility to expansion and contraction, in the following ratio of percentages by weight and volume of the ingredients employed:

40 Preservative-binder, by volume 25 to 40%  
Wood particles, by volume 60 to 75%  
Preservative-binder, by weight 30 to 65%  
Wood particles, by weight 35 to 70%

45 In practice I have discovered that my method of shredding wood into particles of various predetermined sizes and shapes, each particle composed of a plurality of fibers naturally joined together in indiscriminate fashion, results in inter-locking with each other during their contraction, under final compression, and in a distinct advantage, in this regard, over the use of woody particles of approximately uniform size and shapes 50 now employed in such compositions.

The durability of any paving structure depends on: (a) the extent to which the binder is present consistent with its practical agglomeration in the aggregate, in order that the life of the binder may be enhanced by its uniform activity under the action of traffic; (b) the extent the binder penetrates the particles bound thereby, (c) the efficiency of the mechanical clasp between the bound particles, (d) the extent of

voids between, and of unfilled pores within such bound particles, and consequent degrees of density, resiliency, expansion and contraction of the ingredients forming it.

My invention provides the means for (a) fixing the exact quantities essential to be known for such agglomeration of the ingredients of my composition by predetermining the extent of such pores and voids and of the inevitable expansion and contraction thereof; (b) for maximum penetration of the bound particles by the binder that coats them, so that the binder and filler of the voids extends from the core of one particle to the core of all others; (c) for improved mechanical clasp between the particles by reason of the variety in shape thereof, causing interlocking with each other during definite contraction under gradual compression, when cooling, which compression is fixed in point of degree and of time, with relation to such contraction; (d) permanent density and resiliency by the use of woody particles practically graded in various predetermined sizes, in combination with the use of the exact proportions of such ingredients so predetermined in quantity.

In view of the degree of penetration of the woody particles by their binder evidenced by my process, stone and sand used in paving structures are comparatively non-absorbent; cork also used in such compositions will not absorb its binder but is merely surrounded and bound by it; the absorbing efficiency of saw-dust and other woody particles such as those specified in accord with the process disclosed in my issued Patent No. 1,040,321, of 1912, heretofore used in such paving compositions is limited by its ability to absorb the binder.

In the drawings, Fig. 2 is a cross sectional view of a new wearing surface, the product of my invention, laid over and old pavement, in which A represents compressed earth, B old concrete base, C sand cushion for D the worn brick surface. E represents the fibrous composition constructed in sheet form, the subject of this invention.

Fig. 3 is a cross sectional view showing resurfacing of a type of country road in which A designates the earth foundation, B a worn surface of sand-clay or other mixture, while C designates the fibrous composition, the subject of this invention.

Fig. 4 designates a cross section of a worn concrete or Macadam pavement structure, in which A represents the concrete of Macadam structure, and B the fibrous composition the subject of this invention.

Fig. 5 is a cross sectional view of my 125 pavement structure in which the composition is designated by B laid in sheet form on compressed earth foundation A, for country road purposes.

Fig. 6 is a cross sectional view of a city 130

pavement in which A designates the earth foundation, B concrete, D, a layer of fibrous composition the subject of this invention, crowned by E, the subject of this invention 5 formed into blocks. C designates the paint course between the concrete and fibrous composition.

What I claim is:

1. The process of manufacturing a composition of matter from woody particles consisting in first shredding the wood into particles of various predetermined shapes and sizes, extracting therefrom all sap, pulp and matter other than a plurality of woody 10 fibers forming each particle, abnormally enlarging the particles and then partially drying them; then separating the particles in descending gradations of sizes ranging from  $\frac{3}{16}'' \times \frac{1}{8}''$  to  $\frac{1}{16}'' \times \frac{3}{8}''$  and from  $\frac{1}{16}'' \times \frac{3}{8}''$  to  $\frac{1}{4}'' \times \frac{1}{8}''$  15 in minor percentage of their aggregate, mixed with the major volume in sizes graduating from  $\frac{1}{4}'' \times \frac{1}{8}''$  to impalpable dust, the latter representing from 2 to 3% of the aggregate; then measuring and mixing them together in such proportions that their volume 20 will be equivalent to from 70 to 90% of their ungraded volume; then mixing the particles with a binder of preservative nature, preheated to approximately 300 degrees 25 Fahr., then agitating the mass in the presence of sufficient heat sustained a sufficient length of time to exhaust the absorbing efficiency of the particles, simultaneously partially filling the expanded pores with the 30 binder; then exposing the mass, when at a temperature of 250 degrees Fahr., to a cooling temperature to contract the ingredients to normal, simultaneously entrapping the binder within, to the extent of completely 35 filling, the contracting pores, then gradually 40 compressing the mass, while cooling, to 50% of its expanded volume, the quantity of such binder being predetermined in exact relation to measured expansion, contraction 45 and compression of the ingredients, and being merely sufficient to exactly fill the pores of the particles and the voids between the particles in the finished product, and to bind them to each other.
- 50 2. The process of manufacturing a paving composition from variously shaped, abnormally enlarged woody particles of graded sizes, from which have been removed all sap and pulp and the major portion of their moisture content, consisting in then mixing the particles with a binder of preservative 55 nature, pre-heated to 300 degrees Fahr., and then agitating the mass in the presence of sustained heat sufficient to raise the temperature of the mass to 250 degrees Fahr., and 60 to completely develop the absorbing efficiency of the particles, simultaneously partially filling the expanded pores therewith, and then completely filling them when contracting, by entrapping the binder therein, 65 which binder is in quantity predetermined in exact relation to the measured degree of the ingredients' enlargement from and contraction to normal, then gradually compressing the mass to 50% of its expanded volume, simultaneously exuding the binder from the pores of the particles in sufficient quantity to fill the voids between them and to bind them to each other.
- 70 3. A new plastic composition comprising woody particles of various shapes and graded sizes from which sap, pulpy matter and moisture have been removed, mixed with a binder of preservative nature in proportionate quantities predetermined in the following ratio, when cold: binder, by volume 75 80 25 to 40%, wood, by volume 60 to 75%, binder, by weight, 30 to 65%, wood, by weight 35 to 70%.
- 85 4. A new plastic composition comprising woody particles of various shapes and graded sizes, from which sap, pulpy matter and moisture have been removed, mixed under the influence of heat with a binder of preservative nature in quantity predetermined 90 in relation to measured voids within and between the particles.
- 95 5. The method of manufacturing a new pavement structure consisting in mixing variously shaped woody particles, of graded sizes, from which have been removed sap, pulp and moisture, with a binder of preservative nature in the presence of heat, and then spreading the mixture at a temperature of approximately 250 degrees Fahr., 100 not exceeding four inches thick, on a previously prepared road base, and gradually compressing the same to 50% of its hot volume, the quantity of such binder employed having been determined on the following basis: by measuring the pores within and 105 voids between the woody particles when so treated, expanded and grafted, then deducting from 100 the figure representing the aggregate volume of such pores and voids, thereby determining the percentage of solids; 110 then deducting the latter percentage from 50 and to the resulting figure adding from seven to ten per cent.

In testimony whereof, I have affixed my 115 signature in the presence of two witnesses, the 16th day of June 1914.

GEORGE ASA HENDERSON.

Witnesses:

R. C. SWEET,  
O. B. MELTON.